

Oct. 5, 1926.

1,602,286

G. M. SMITH

ORNAMENTAL MATERIAL AND METHOD OF PREPARING THE SAME

Filed March 3, 1926

*Fig. 1.*



*Fig. 2.*



INVENTOR.

*Gordon M. Smith*  
BY  
*Emery, Booth, James & Nancy* ATTORNEYS.

## UNITED STATES PATENT OFFICE.

GARDNER M. SMITH, OF ST. LOUIS, MISSOURI.

## ORNAMENTAL MATERIAL AND METHOD OF PREPARING THE SAME.

Application filed March 3, 1926. Serial No. 92,091.

This invention relates to the art of ornamentation and has as an object to provide an ornamental sheet material, and a method of preparing the same.

5 Other objects and advantages of the invention will appear hereinafter.

Many open work fabrics such as lace, for example, while highly ornamental, have not been widely used for surface ornamentation 10 because their delicate structure is too fragile to withstand hard usage, and also because of the difficulty of securing such fabrics to a surface.

According to the present invention, it is 15 proposed to apply lace or similar open work fabrics to a backing sheet of leather, thus forming a composite sheet suitable for use in many relations. For example, such sheet material could be used to advantage in 20 the making of uppers for ladies' shoes, or, indeed, wherever leather is used as an outer covering for decorative as well as utilitarian purposes.

A preferred embodiment of the invention 25 selected for purposes of illustration is shown in the accompanying drawings, in which,

Figure 1 is a top plan view of the assembled sheet material, and

30 Figure 2 is a greatly enlarged sectional view.

According to the preferred method of preparing the composite sheet, a sheet or strip of lace 1 is laid over a sheet of leather 35 2, the two sheets being held and supported face to face by any suitable means. A coating of cementitious material, preferably colorless, is then applied to the assembled sheets in sufficient quantity to thoroughly 40 saturate and impregnate the lace, and to secure the individual strands or filaments thereof tightly to the leather.

While the invention is not limited to the use of any particular cementitious material, 45 it has been found that a pyroxylin cement such as a butyl acetate cellulose nitrate solution is particularly well adapted for the purpose, for it is substantially colorless and provides a thin waterproof coating over 50 both leather and fabric which serves to protect both to a certain degree.

After the cement has set, the composite sheet may be pressed to smoothness by the application of heat and pressure, or if desired, for special purposes, the composite

sheet may be embossed by ordinary methods.

If desired, the leather sheet may be stretched somewhat and may be held in stretched condition while the cement is applied, in order to open the pores to permit 60 penetration of the cement to cause better adhesion. It is not ordinarily desirable to stretch the lace, it being sufficiently merely to lay it flat against the surface of the leather.

For certain purposes, as where the composite sheet is to be subjected to severe flexing, the lace may be dipped in or treated with a suitable lubricant such as castor-oil 70 prior to the application of the cement.

The finished sheet is substantially as flexible as the leather backing sheet to which the lace is applied, and may be handled and worked in substantially the same manner. Due to the impregnation of the cement, 75 however, the lace becomes much more durable and less susceptible to destruction when subjected to scuffing such as is ordinarily received by shoe uppers.

While the cement applied forms a protective coating over the leather and lace which is sufficient for most purposes, for special purposes, as where the outer surface of the material is to be subjected to very severe scuffing, an additional film or coating 85 of pyroxylin may be applied.

It will be understood that the invention may be variously modified and embodied within the scope of the subjoined claims.

I claim as my invention:

1. The method of ornamenting leather sheets which comprises treating a sheet of lace with lubricant, and cementing the same to the leather sheet.

2. A composite ornamental sheet comprising a leather body portion having a superficial layer of openwork textile fabric cemented thereto, the strands of said openwork fabric standing out in relief above the surface of the leather.

3. A composite ornamental sheet comprising a leather body portion having a superficial layer of openwork textile fabric cemented thereto by a transparent waterproof cement, the strands of said openwork fabric standing out in relief above the surface of the leather.

4. A composite ornamental sheet comprising a leather body portion having a superficial layer of openwork textile fabric

110

cemented thereto by a transparent pyroxylin composition, the strands of said openwork fabric standing out in relief above the surface of the leather.

5. The method of making ornamental composite sheets comprising assembling an openwork textile fabric and a leather sheet in superimposed relation, and applying a cementitious waterproof material in sufficient quantity to saturate and impregnate the fabric and to cause it to adhere firmly to the surface of the leather.
- 10 6. The method of making ornamental

composite sheets comprising assembling an openwork textile fabric and a leather sheet in superimposed relation, applying a cementitious waterproof material in sufficient quantity to saturate and impregnate the fabric and to cause it to adhere firmly to the surface of the leather and applying smoothing pressure and heat to remove the wrinkles after the cement has set.

In testimony whereof, I have signed my name to this specification this 26th day of February, 1926.

GARDNER M. SMITH.